# EUROPEAN PATENT SPECIFICATION

(11) **EP 4 212 639 B1**
(45) Date of publication and mention of the grant of the patent: **04.06.2025**
(21) Application number: 22202560.3
(22) Date of filing: 19.10.2022
(51) Int. Cl.: C22C 19/05, F01D 5/28, F01D 25/00, F01D 25/24

(54) **NICKEL-BASED ALLOY AND TURBINE WHEEL INCORPORATING SAME**
NICKELBASIERTE LEGIERUNG UND TURBINENRAD DAMIT
ALLIAGE À BASE DE NICKEL ET ROUE DE TURBINE L'INCORPORANT

(30) Priority: 18.01.2022 IN 202211002807; 21.03.2022 US 202217655565
(43) Date of publication of application: 19.07.2023
(73) Proprietor: Garrett Transportation I Inc., Torrance, CA 90504 (US)
(72) Inventor: Ricankova, Veronika, Torrance, 90504 (US); Kannusamy, Ragupathy, Torrance, 90504 (US); Wilson, Marc, Torrance, 90504 (US); Renaud, Philippe, Torrance, 90504 (US); Morrissey, Michael, Torrance, 90504 (US); Chimangala Seetharamrao, Prashanth, Torrance, 90504 (US)
(74) Representative: LKGlobal UK Ltd.

(56) References cited:
- EP-A1- 2 805 784
- US-A- 5 611 670

## Description

### CROSS-REFERENCE TO RELATED APPLICATIONS

This application is related to and claims all available benefit of Indian Provisional Patent Application IPA: 202211002807 filed January 18, 2022.

### TECHNICAL FIELD

The present disclosure is generally directed to metal alloys with improved high-temperature oxidation and fatigue resistance for use in turbocharger applications. More particularly, the present disclosure is directed to nickel-based alloys and turbine wheels including nickel-based alloys.

### BACKGROUND

Turbochargers for gasoline and diesel internal combustion engines are devices known in the art that are used for pressurizing or boosting the intake air stream, routed to a combustion chamber of the engine, by using the heat and volumetric flow of exhaust gas exiting the engine. Specifically, the exhaust gas exiting the engine is routed into a turbine housing of a turbocharger in a manner that causes an exhaust gas-driven turbine wheel to spin within the housing. The exhaust gas-driven turbine wheel is mounted onto one end of a shaft that is common to a radial air compressor mounted onto an opposite end of the shaft and housed in a compressor housing. Thus, rotary action of the turbine wheel also causes the air compressor to spin within a compressor housing of the turbocharger that is separate from the turbine housing. The spinning action of the air compressor causes intake air to enter the compressor housing and be pressurized or boosted a desired amount before it is mixed with fuel and combusted within the engine combustion chamber.

The turbine wheel, usually a cast nickel-based alloy, used in turbochargers is a highspeed rotating component that is exposed to high temperature combustion gasses between temperatures of about 750°C to about 1050°C, depending upon the application. To withstand such a high temperature, the nickel-based alloy material should be oxidation resistant, creep resistant as well as thermo-mechanical fatigue resistant while rotating in the approximately 100,000 - 300,000 RPM range. Existing alloys for such applications all have various deficiencies: For example, the Mar-M-246 nickel-based alloy is relatively expensive, whereas the IN-713C nickel-based alloy exhibits inferior high-temperature properties.

Therefore, it will become apparent to those skilled in the art that there remains a present and continuing need for the provision of improved nickel-based alloys and turbine wheels that include such nickel-based alloys. Particularly, it would be desirable to provide an alloy based on Mar-M-246 but with an improved chemistry that reduces costs significantly while still retaining the desirable high-temperature oxidation and corrosion, creep and thermo-mechanical fatigue resistance, for example, of Mar-M-246. Furthermore, other desirable features and characteristics of the inventive subject matter will become apparent from the subsequent detailed description of the inventive subject matter and the appended claims, taken in conjunction with the accompanying drawings and this background of the disclosure. Documents cited during prosecution include US 5 611 670 A and EP 2 805 784 A1.

### BRIEF SUMMARY

Nickel-based alloys and turbocharger turbine wheels including nickel-based alloys are disclosed herein. The nickel-based alloy according to the invention is defined in the appended claims. Additionally, in some examples (although an amount of 0.00% of any of the following elements may be present), the nickel-based alloy may include or further consist of tantalum in an amount of less than about 0.10%, manganese in an amount of less than about 0.03%, silicon in an amount of less than about 0.03%, iron in an amount of less than about 1.00%, copper in an amount of less than about 0.02%, sulfur in an amount of less than about 10 ppm and phosphorous in an amount of less than about 50 ppm.

With regard to the foregoing alloy embodiments: the amount of cobalt may be limited to about 2.25% to about 2.75%; alternatively or additionally, the amount of chromium may be limited to about 12.00% to about 12.80%; alternatively or additionally, the amount of aluminum may be limited to about 6.40% to about 6.80%; alternatively or additionally, the amount of tungsten may be limited to about 5.25% to about 5.75%; alternatively or additionally, the amount of molybdenum may be limited to about 2.40% to about 2.60%; alternatively or additionally, the amount of titanium may be limited to about 1.35% to about 1.65%; alternatively or additionally, the amount of niobium may be limited to about 0.80% to about 1.20%.

In another exemplary embodiment, a turbocharger turbine wheel includes or consists of, at least as a part of its overall composition, a nickel-based alloy as defined in the appended claims. Such a turbine wheel may find application for operating at temperatures from 980°C to 1020°C.

With regard to the foregoing turbine wheel embodiments: the amount of cobalt may be limited to about 2.25% to about 2.75%; alternatively or additionally, the amount of chromium may be limited to about 12.00% to about 12.80%; alternatively or additionally, the amount of aluminum may be limited to about 6.40% to about 6.80%; alternatively or additionally, the amount of tungsten may be limited to about 5.25% to about 5.75%; alternatively or additionally, the amount of molybdenum may be limited to about 2.40% to about 2.60%; alternatively or additionally, the amount of titanium may be limited to about 1.35% to about 1.65%; alternatively or additionally, the amount of niobium may be limited to about 0.80% to about 1.20%.

This brief summary is provided to introduce a selection of concepts in a simplified form that are further described below in the detailed description and the drawings. This summary is not intended to identify key features or essential features of the claimed subject matter, nor is it intended to be used as an aid in determining the scope of the claimed subject matter.

### BRIEF DESCRIPTION OF THE DRAWING

The various embodiments will hereinafter be described in conjunction with the following drawing figures, wherein like numerals denote like elements, and wherein:
FIG. 1 illustrates a system view of an exemplary internal combustion engine including a turbocharger having a turbine wheel in accordance with some embodiments of the present disclosure;
FIG. 2 illustrates a partial view of a turbine wheel including blades with cracks formed via hot tearing phenomenon in accordance with some embodiments of the present disclosure;
FIG. 3 illustrates an enlarged view of a microstructure examination of a crack formed in one of the blades of the turbine wheel depicted in FIG. 2;
FIG. 4 illustrates a partial view of a turbine wheel that failed from fatigue due to a blade that had a pre-existing defect (crack(s)) formed via hot tearing phenomenon in accordance with some embodiments of the present disclosure;
FIG. 5 illustrates a graphical representation of freezing ranges of various alloys including an improved nickel-based alloy in accordance with some embodiments of the present disclosure;
FIG. 6 illustrates a graphical representation of solid and liquid fractions as a function of temperature at a heating/cooling rate of 1°K of various alloys including an improved nickel-based alloy in accordance with some embodiments of the present disclosure;
FIG. 7 illustrates a castability analysis of a turbine wheel formed from MarM246 alloy showing the probability of occurrence of cracks formed via hot tearing phenomenon;
FIG. 8 illustrates a castability analysis of a turbine wheel formed from an improved nickel-based alloy showing the probability of occurrence of cracks formed via hot tearing phenomenon in accordance with some embodiments of the present disclosure;
FIG. 9 illustrates a graphical representation of computed densities as a function of temperature of various alloys including an improved nickel-based alloy in accordance with some embodiments of the present disclosure;
FIG. 10 illustrates a graphical representation of computed moduli as a function of temperature of various alloys including an improved nickel-based alloy in accordance with some embodiments of the present disclosure; and
FIG. 11 illustrates a graphical representation of gamma prime volume fractions at different temperatures of various alloys including an improved nickel-based alloy in accordance with some embodiments of the present disclosure.

### DETAILED DESCRIPTION

The following detailed description is merely exemplary in nature and is not intended to limit the invention or the application and uses of the invention. As used herein, the word "exemplary" means "serving as an example, instance, or illustration." Thus, any embodiment described herein as "exemplary" is not necessarily to be construed as preferred or advantageous over other embodiments. All of the embodiments described herein are exemplary embodiments provided to enable persons skilled in the art to make or use the invention and not to limit the scope of the invention which is defined by the claims. Furthermore, there is no intention to be bound by any expressed or implied theory presented in the preceding technical field, background, brief summary, or the following detailed description.

Unless specifically stated or obvious from context, as used herein, the term "about" is understood as within a range of normal tolerance in the art, for example within 2 standard deviations of the mean.

Embodiments of the present disclosure provide an improved nickel-based alloy and turbocharger turbine wheels made with this nickel-based alloy. The disclosed embodiments detail an improved nickel-based alloy chemistry that is less expensive than Mar-M-246 yet has better high-temperature properties as compared with IN-713C.

With reference now to FIG. 1, illustrated is a turbocharger 101 in accordance with the present disclosure having a radial turbine and that includes a turbocharger housing and a rotor configured to rotate within the turbocharger housing along an axis of rotor rotation 103 on thrust bearings and two sets of journal bearings (one for each respective rotor wheel), or alternatively, other similarly supportive bearings. The turbocharger housing includes a turbine housing 105, a compressor housing 107, and a bearing housing 109 (*i.e.,* a center housing that contains the bearings) that connects the turbine housing 105 to the compressor housing 107. The rotor includes a turbine wheel 111 located substantially within the turbine housing 105, a compressor wheel 113 located substantially within the compressor housing 107, and a shaft 115 extending along the axis of rotor rotation 103, through the bearing housing 109, to connect the turbine wheel 111 to the compressor wheel 113.

The turbine housing 105 and turbine wheel 111 form a turbine configured to circumferentially receive a high-pressure and high-temperature exhaust gas stream 121 from an engine, *e.g*., from an exhaust manifold 123 of an internal combustion engine 125. The turbine wheel 111 (and thus the rotor) is driven in rotation around the axis of rotor rotation 103 by the high-pressure and high-temperature exhaust gas stream 121, which becomes a lower-pressure and lower-temperature exhaust gas stream 127 and is axially released into an exhaust system (not shown).

The compressor housing 107 and compressor wheel 113 form a compressor stage. The compressor wheel 113, being driven in rotation by the exhaust-gas driven turbine wheel 111, is configured to compress axially received input air (*e.g.,* ambient air 131, or already-pressurized air from a previous-stage in a multi-stage compressor) into a pressurized air stream 133 that is ejected circumferentially from the compressor. Due to the compression process, the pressurized air stream is characterized by an increased temperature over that of the input air.

Optionally, the pressurized air stream may be channeled through a convectively cooled charge air cooler 135 configured to dissipate heat from the pressurized air stream 133, increasing its density. The resulting cooled and pressurized output air stream 137 is channeled into an intake manifold 139 on the internal combustion engine, or alternatively, into a subsequent-stage, in-series compressor. The operation of the system is controlled by an engine control unit (ECU) 151 that connects to the remainder of the system via communication connections 153.

The composition of an exemplary nickel-based alloy is now provided below with respect to its constituent elements (all percentages being provided on a weight basis of the overall alloy composition, unless otherwise noted). In one embodiment, elements that are associated with grain boundary cracking and embrittlement should be minimized. For example, in this embodiment, the content of silicon (Si) is maintained below or equal to about 0.03%. The content of phosphorous (P) is maintained below or equal to about 50 ppm. Further, the content of sulfur (S) is maintained below or equal to about 10 ppm. As an additional matter, to reduce cracking, the master heat alloy that is used to process the alloy to ingot form desirably does not contain any casting revert or scrap having detrimental tramp or trace elements.

Elements that are associated with grain boundary strengthening, including carbon (C), boron (B), and zirconium (Zr) are melting point depressants which can create hot cracks during solidification in a casting process (hot tearing phenomenon) and welding (solidification cracking) of alloys. Grain boundary liquation during welding of alloys is linked to carbides and borides. Since C (but not B) achieves a "carbon boil" during master alloy refining, embodiments of the nickel-based alloy retain some carbon, likely in the form of carbides (as described below) but not a significant content of borides. Zr or B does not influence the castability when added individually. However, when both Zr and B are present in the alloy, high hot tearing susceptibility was found, the effect being particularly strong if Zr concentration was high. Accordingly, the content of B is maintained in a range of about 0.01% to about 0.02%, the content of carbon is maintained in a range of about 0.13% to about 0.17%, and the content of zirconium is maintained in a range of about 0.03% to about 0.05%.

With the aforementioned relatively lower C and B content, the undesirable formation of topologically close-packed (TCP) brittle phases requires concomitant lowering of the minimum amounts of several refractory elements known to form TCP phases. For example, chromium (Cr), molybdenum (Mo), cobalt (Co), and tungsten (W) can combine to form TCP phases. Of these, reducing the Cr lower limit is desirably avoided because Cr plays a role in oxidation/sulfidation resistance. Accordingly, the content of Cr is from 12.0% to about 14.0%. In another embodiment, the content of Cr is from about 12.0% to about 12.8%.

Co is a solid solution strengthening element, but it can contribute to TCP phase formation. Accordingly, permitting a lower Co content has been discovered to be beneficial from lower risk of TCP formation, lower density and lower cost point of view. Thus, the content of Co is from about 2.00% to about 3.00%. In another embodiment, the content of Co is from about 2.25% to about 2.75%.

Furthermore, W is known to be an element that forms carbides, that acts as a solid solution strengthening element, and that forms TCP phases especially in case of high percentage of gamma prime in alloys. W is also a relatively expensive element and increases density of alloys. Accordingly, permitting a lower W content has been discovered to be beneficial. Thus, the content of W is from about 5.00% to about 6.00%. In another embodiment, the content of W is from about 5.25% to about 5.75%.

Titanium (Ti) is both a carbide and gamma-prime phase forming element. The gamma-prime phase is favorable for high-temperature oxidation resistance. Gamma-prime phase volume fraction and its thermal stability at high temperature is key for alloys for higher mechanical properties, creep and thermo-mechanical fatigue resistance during severe thermal-shock loading conditions. Accordingly, titanium is provided in a range of about 1.25% to about 2.00%. In other embodiments, titanium is provided in a range of about 1.35% to about 1.65%.

Mo is a solid solution strengthening element and increases the Al partitioning to the gamma-prime phase by reducing the solubility of Al in the γ matrix which increases gamma-prime volume fraction. Moreover, Mo is known to be an element that forms primary MC carbides and that forms detrimental phases like TCP phases or M₆C carbides, in some instances, the formation of M₆C is an intragranular Widmanstatten precipitates. Alloy tends to precipitate M6C carbides if the alloy has a sufficiently high molybdenum + tungsten content (Mo + ½W ≥6 wt%). There is evidence in the art that Mo may be detrimental to hot corrosion or oxidation resistance. Mo oxide volatility may also be a negative factor. Moderate-strength cast alloys such as IN-738 and higher-strength cast alloys such as IN-792 have achieved greatly improved corrosion resistance with low levels of molybdenum and tungsten, and beneficial levels of chromium (12 to 15%). Accordingly, the content of Mo is maintained within a range of about 2.25% to about 2.75%. In another embodiment, the content of Mo is maintained with a range of about 2.40% to about 2.60%.

Continuing with the description of an exemplary embodiment of the nickel-based alloy, niobium (Nb) is known to be an element that forms carbides and a solid solution strengthening element that also partitions to the gamma-prime phase. The phase fraction and stability of γ' increases with niobium content. Allowing a higher content of Nb will favor Nb-rich carbides and make up for the absence of Ti in the gamma-prime phase while contributing to solid solution strengthening. Moreover, Nb is preferred MC carbide former because titanium-rich MC carbides are less stable and introduce deleterious M₆C reactions. Accordingly, the content of Nb is from about 0.55% to about 1.50%. In another embodiment, the content of Nb is from about 0.80% to about 1.20%.

Al, as a gamma-prime phase forming element, is also included in the alloy composition of the present disclosure. The content of Al is from about 5.75% to about 6.85%. In another embodiment, the content of Al is from about 6.40% to about 6.80%.

Other elements that may be present in small amounts (or possibly 0%) in some embodiments include tantalum (Ta) in an amount of less than about 0.10%, manganese (Mn) in an amount of less than about 0.03%, iron (Fe) in an amount of less than about 1.00%, and copper (Cu) in an amount of less than about 0.02%.

Moreover, as the described alloys are nickel-based, it will be appreciated that nickel (Ni) forms a majority of the content (*i.e.,* greater than about 50%) of the described alloy. That is, nickel accounts for the balance of the content not otherwise described above, while accounting for inevitable/unavoidable impurities not otherwise set forth above as are commonly understood in the art.

Table 1, set forth below, provides the elemental content of a nickel-based alloy of the present disclosure in accordance with the description provided above, while also specifying the maximum content of additional detrimental tramp or trace elements commonly encountered in nickel-based alloys. Each weight percentage included in Table 1 is understood to be preceded by the term "about." In addition, a minimum of zero, signified by "<", means "low as possible", not to exceed the maximum. It should be acknowledged that trace amounts of inevitable/unavoidable impurities may be present (in trace amounts), although not explicitly listed in Table 1, as is known in the art.

**TABLE 1**

| Application Temperature (C) | 980°C-1020°C |
|---|---|
| Chemical Element | % |
| Carbon, C | 0.13-0.17 |
| Manganese, Mn | <0.03 |
| Sulfur, S | <10 ppm |
| Silicon, Si | <0.03 |
| Chromium, Cr | 12.0-14.0 |
| Molybdenum, Mo | 2.25-2.75 |
| Tungsten, W | 5.00-6.00 |
| Titanium, Ti | 1.25-2.00 |
| Boron, B | 0.01-0.02 |
| Niobium, Nb | 0.55-1.50 |
| Aluminum, Al | 5.75-6.85 |
| Zirconium, Zr | 0.03-0.05 |
| Cobalt, Co | 2.00-3.00 |
| Iron, Fe | <1.00 |
| Tantalum, Ta | <0.10 |
| Copper, Cu | <0.02 |
| Phosphorous, P | <50 ppm |
| Nickel, Ni | Balance |

As such, described herein are embodiments of improved nickel-based alloys and turbocharger turbine wheels made with such nickel-based alloys. The described embodiments provide a high-temperature oxidation and corrosion resistance, creep and thermo-mechanical fatigue resistant and very good castable (due to lower freezing range and density) nickel-based alloy that is achieved, in part, with increased in chromium and aluminum, significantly decreased tungsten and cobalt, addition of niobium, with no tantalum, in comparison to Mar-M-246. The resultant alloy has a reduced cost, wherein the raw material is about 15% less than Mar-M-246. Thus, the novel alloy described herein will have good mechanical properties, better creep and thermo-mechanical fatigue resistance, better oxidation/hot corrosion resistance and better castability with lesser density and cost, and will be a suitable alternative to the prior art options. As such, the alloy of the present disclosure can be used to make turbine wheels for applications reaching temperatures from 980°C to 1020°C with lower cost than existing commercial alloys.

### ILLUSTRATIVE EXAMPLES

The present disclosure is now illustrated by the following non-limiting examples. It should be noted that various changes and modifications can be applied to the following examples and processes without departing from the scope of this invention, which is defined in the appended claims. Therefore, it should be noted that the following examples should be interpreted as illustrative only and not limiting in any sense.

FIG. 2 illustrates a partial view of a turbine wheel including blades with cracks formed via hot tearing phenomenon. FIG. 3 illustrates an enlarged view of a microstructure examination of a crack formed in one of the blades of the turbine wheel.

Hot tearing (HTR) phenomenon, also referred to as hot cracking or hot shortness, represents the formation of an irreversible failure (crack) in the still semisolid casting during formation via casting of a metal alloy part. Hot tearing arises from a complex combination of thermal-mechanical and solidification phenomena, basically being associated with the incomplete liquid feeding and tensile stress generated in coherent regions of mushy zones, more specifically, in areas with a high solid fraction of 0.9 and beyond. It is generally believed that hot tearing occurs above the solidus temperature when the volume fraction of solid is, for example, 85% to 95% and the solid phase is organized in a continuous network of grains and propagates in the interdendritic and/or intergranular liquid film. "Time spend" in mushy zone during solidification is possible to influence by the chemical composition of the alloy.

As illustrated, due to the complexity of the turbine wheel, particularly the changes of cross-sectional dimensions of the blades, cracks can occur in the blades by casting turbine wheels. There may be multiple factors that could be involved in the formation of cracks at supersolidus temperatures, however a primary cause is inadequate compensation of solidification shrinkage by melt flow in the presence of thermal stresses. These cracks can be difficult to detect visually or by non-destructive analysis (NDA) and, as such, can result in some cast parts being used in the field, which may have a shorted "use life."

FIG. 4 illustrates a partial view of a turbine wheel that failed from fatigue due to a blade that had a pre-existing defect (crack(s)) formed via hot tearing phenomenon. The fatigue damage was generated from (1) vibrations produced during operation of the turbine wheel and (2) change of strain distribution due to: (a) stress concentration (e.g., notch or pre-existing defect/crack acts as a stress concentrator) and/or (b) deflection distribution or change of blade movement also referred to as a "Flag effect."

Example metal alloys (referred to herein as "MarM246" and "G246UL") with the following compositions were used in the examples presented below in Table 2 with respect in FIGS. 5-11. "MarM246" represents an existing nickel-based alloy and "G246UL" represents an improved nickel-based alloy in accordance with some embodiments of the present disclosure.

FIG. 5 illustrates a graphical representation of freezing ranges of various alloys including Inconel 713C (another existing nickel-based alloy) and MarM246 and G246UL referenced above. Specifically, the freezing range is the solidification temperature range between an alloy's liquidus and solidus phases. This temperature range has impact on HTR occurrence risk and reducing the freezing temperature range is critical for reducing the HTR occurrence risk. The HTR occurrence risk is bigger with wider freezing range especially with longer time spend in mushy zone. Faster solidification helps decrease HTR risk. Freezing range and solidification temperature of remaining liquid is affected by the chemical composition of the alloy.

ThermoCalc software was used for computation of the freezing range of Mar-M-246, Inconel 713C and G246UL. Precision of computation was reviewed by experimental measurement of Mar-M-246 and Inconel 713C by DSC (Differential scanning calorimetry) equipment. Correlation between computation and experimental measurement was found to be very good.

As illustrated, G246UL exhibits similar, but slightly lower, computed values of freezing range to Inconel 713C and much lower in comparison to Mar-M-246. Further, it was observed that Inconel 713C castability is better and HTR occurrence is much lower in comparison to Mar-M-246. As such, castability of G246UL is better and HTR occurrence is much lower in comparison to Mar-M-246 and correspondingly improved over Inconel 713C.

FIG. 6 illustrates a graphical representation of solid and liquid fractions as a function of temperature at a heating/cooling rate of 1°K (e.g., cooling rate as part of a casting process) of Mar-M-246 and G246UL. As illustrated, G246UL exhibits tighter freezing range and tighter temperature range "spend" in mushy zone, indicating a much lower probability of HTR occurrence in comparison to Mar-M-246.

FIGS. 7-8 illustrates a castability analysis of a turbine wheel formed from MarM246 alloy and G246UL, respectively, showing the probability of occurrence of cracks formed via hot tearing phenomenon. Notably the Hot Tear Index scale in FIG. 8 is divided by 2 in comparison to the Hot Tear Index scale in FIG. 7. As illustrated, G246UL gives lower HTR risk (i.e., a much lower probability of HTR occurrence) compared to MarM246 due to differences in chemical compositions. In particular, the probability of HTR occurrence at various locations (#1-#4) on the blades of the respective turbine wheel is provided in the table (Table 3) below:

FIG. 9 illustrates a graphical representation of computed densities as a function of temperature of Inconel 713C, MarM246, and G246UL. FIG. 10 illustrates a graphical representation of computed moduli as a function of temperature of Inconel 713C, MarM246, and G246UL. Density and Modulus were computed for G246UL with JMatPro and compared with Mar-M-246 and Inconel 713C experimental data. Computed modulus of G246UL is similar to Mar-M-246 at temperatures above 900°C and higher than Inconel 713C. As previously discussed, the operating temperature of a turbine wheel is above 900°C and the higher modulus is desirable at operating temperatures because it helps reduce the likelihood of any fatigue damage generated from a change of strain distribution during operation due to, for example, deflection distribution or change of blade movement, also referred to as a "Flag effect."

Further, the computed density of G246UL is lower than MM246, which can provide a benefit in the case of turbine wheel inertia and will be beneficial in case of material castability. It is believed that lower density is better for castability.

FIG. 11 illustrates a graphical representation of gamma prime volume fractions at different temperatures of G246UL and MM246. In particular, ThermoCalc software was used for computation of phase diagrams of Mar-M-246 and G246UL. Gamma prime volume fraction at different temperatures (900°C, 950°C and 1000°C) were taken for materials comparison. Gamma prima volume fraction and its thermal stability at high temperatures is important for an alloy's mechanical properties and creep, fatigue, thermo-mechanical fatigue resistance during operation at high temperatures. Gamma prima volume fraction of from about 55 to about 75 at high temperatures of 900°C, 950°C and 1000°C are preferred. As illustrated, G246UL exhibits higher gamma prime volume fraction, from about 58 to about 68, at high temperatures compared to about 52 to about 64 of Mar-M-246.

While at least one exemplary embodiment has been presented in the foregoing detailed description of the invention, it should be appreciated that a vast number of variations exist. It should also be appreciated that the exemplary embodiment or exemplary embodiments are only examples, and are not intended to limit the scope, applicability, or configuration of the invention in any way. Rather, the foregoing detailed description will provide those skilled in the art with a convenient road map for implementing an exemplary embodiment of the invention, it being understood that various changes may be made in the function and arrangement of elements described in an exemplary embodiment without departing from the scope as set forth in the appended claims.

## Claims

1. A nickel-based alloy, wherein the nickel-based alloy comprises, on a weight basis of the overall alloy:
2.00% to 3.00% cobalt,
12.0% to 14.0% chromium,
5.75% to 6.85% aluminum,
5.00% to 6.00% tungsten,
2.25% to 2.75% molybdenum,
1.25% to 2.00% titanium,
0.55% to 1.50% niobium,
0.13% to 0.17% carbon,
0.03 to 0.05% zirconium,
0.01% to 0.02% boron,
optionally, tantalum in an amount of less than 0.10%,
manganese in an amount of less than 0.03%,
silicon in an amount of less than 0.03%,
iron in an amount of less than 1.00%,
copper in an amount of less than 0.02%,
sulfur in an amount of less than 10 ppm,
phosphorous in an amount of less than 50 ppm, and
a balance of nickel, with the proviso that inevitable/unavoidable impurities may be present in trace amounts.

2. The nickel-based alloy of claim 1, wherein the amount of cobalt is from 2.25% to 2.75%.

3. The nickel-based alloy of claim 1 or 2, wherein the amount of chromium is from 12.00% to 12.80%.

4. The nickel-based alloy of any preceding claim, wherein the amount of aluminum is from 6.40% to 6.80%.

5. The nickel-based alloy of any preceding claim, wherein the amount of tungsten is from 5.25% to 5.75%.

6. The nickel-based alloy of any preceding claim, wherein the amount of molybdenum is from 2.40% to 2.60%.

7. The nickel-based alloy of any preceding claim, wherein the amount of titanium is from 1.35% to 1.65%.

8. The nickel-based alloy of any preceding claim, wherein the amount of niobium is from 0.80% to 1.20%.

9. A turbocharger turbine wheel comprising a nickel-based alloy, wherein the nickel-based alloy is the nickel based alloy of any preceding claim.

## Patentansprüche

1. Nickelbasierte Legierung, wobei die nickelbasierte Legierung auf Gewichtsbasis der gesamten Legierung Folgendes umfasst:
2,00 % bis 3,00 % Cobalt,
12,0 % bis 14,0 % Chrom,
5,75 % bis 6,85 % Aluminium,
5,00 % bis 6,00 % Wolfram,
2,25 % bis 2,75 % Molybdän,
1,25 % bis 2,00 % Titan,
0,55 % bis 1,50 % Niob,
0,13 % bis 0,17 % Kohlenstoff,
0,03 bis 0,05 % Zirconium,
0,01 % bis 0,02 % Bor,
gegebenenfalls Tantal in einer Menge von weniger als 0,10 %,
Mangan in einer Menge von weniger als 0,03 %,
Silizium in einer Menge von weniger als 0,03 %,
Eisen in einer Menge von weniger als 1,00 %,
Kupfer in einer Menge von weniger als 0,02 %,
Schwefel in einer Menge von weniger als 10 ppm,
Phosphor in einer Menge von weniger als 50 ppm, und
einen Rest aus Nickel unter der Bedingung, dass zwangsläufige/unvermeidliche Verunreinigungen in geringen Mengen vorhanden sein können.

2. Nickelbasierte Legierung nach Anspruch 1, wobei die Menge an Cobalt zwischen 2,25 % und 2,75 % beträgt.

3. Nickelbasierte Legierung nach Anspruch 1 oder 2, wobei die Menge an Chrom zwischen 12,00 % und 12,80 % beträgt.

4. Nickelbasierte Legierung nach einem der vorhergehenden Ansprüche, wobei die Menge an Aluminium zwischen 6,40 % und 6,80 % beträgt.

5. Nickelbasierte Legierung nach einem der vorhergehenden Ansprüche, wobei die Menge an Wolfram zwischen 5,25 % und 5,75 % beträgt.

6. Nickelbasierte Legierung nach einem der vorhergehenden Ansprüche, wobei die Menge an Molybdän zwischen 2,40 % und 2,60 % beträgt.

7. Nickelbasierte Legierung nach einem der vorhergehenden Ansprüche, wobei die Menge an Titan zwischen 1,35 % und 1,65 % beträgt.

8. Nickelbasierte Legierung nach einem der vorhergehenden Ansprüche, wobei die Menge an Niob zwischen 0,80 % und 1,20 % beträgt.

9. Turbinenrad eines Turboladers, das eine nickelbasierte Legierung umfasst, wobei die nickelbasierte Legierung die nickelbasierte Legierung nach einem der vorhergehenden Ansprüche ist.

## Revendications

1. Alliage à base de nickel, dans lequel l'alliage à base de nickel comprend, sur une base pondérale de l'alliage général :
2,00 % à 3,00 % de cobalt
12,0 % à 14,0 % de chrome,
5,75 % à 6,85 % d'aluminium,
5,00 % à 6,00 % de tungstène,
2,25 % à 2,75 % de molybdène,
1,25 % à 2,00 % de titane,
0,55% à 1,50 % de niobium,
0,13 % à 0,17 % de carbone,
0,03 % à 0,05 % de zirconium,
0,01 % à 0,02 % de bore,
en option du tantale dans une quantité inférieure à 0,10 %,
du manganèse dans une quantité inférieure à 0,03 %,
du silicium dans une quantité inférieure à 0,03 %,
du fer dans une quantité inférieure à 1,00 %,
du cuivre dans une quantité inférieure à 0,02 %,
du soufre dans une quantité inférieure à 10 ppm,
du phosphore dans une quantité inférieure à 50 ppm, et
un équilibre de nickel sous réserve que des impuretés inévitables puissent être présentes en quantité à l'état de trace.

2. Alliage à base de nickel selon la revendication 1, dans lequel la quantité de cobalt est de 2,25 % à 2,75 %.

3. Alliage à base de nickel selon la revendication 1 ou 2, dans lequel la quantité de chrome est de 12,00 % à 12,80 %.

4. Alliage à base de nickel selon l'une quelconque revendication précédente, dans lequel la quantité d'aluminium est de 6,40 % à 6,80 %.

5. Alliage à base de nickel selon l'une quelconque revendication précédente, dans lequel la quantité de tungstène est de 5,25 % à 5,75 %.

6. Alliage à base de nickel selon l'une quelconque revendication précédente, dans lequel la quantité de molybdène est de 2,40 % à 2,60 %.

7. Alliage à base de nickel selon l'une quelconque revendication précédente, dans lequel la quantité de titane est de 1,35 % à 1,65 %.

8. Alliage à base de nickel selon l'une quelconque revendication précédente, dans lequel la quantité de niobium est de 0,80 % à 1,20 %.

9. Roue de turbine de turbocompresseur comprenant un alliage à base de nickel, dans lequel l'alliage à base de nickel est l'alliage à base de nickel selon l'une quelconque revendication précédente.
